

# UNITED STATES PATENT OFFICE.

WALTER HAMIS GLOVER, OF BRAINTREE, AND LEONARD PHILIP WILSON, OF COVENTRY, ENGLAND, ASSIGNEES, BY MESNE ASSIGNMENTS, TO THE VISCOS COMPANY, OF MARCUS HOOK, PENNSYLVANIA, A CORPORATION OF PENNSYLVANIA.

## MANUFACTURE AND PRODUCTION OF CELLULOSE COMPOUNDS.

1,279,328.

Specification of Letters Patent. Patented Sept. 17, 1918.

No Drawing.

Application filed January 22, 1915. Serial No. 3,830.

*To all whom it may concern:*

Be it known that we, WALTER HAMIS GLOVER, a subject of the King of Great Britain, residing at The Avenue, Braintree, 5 in the county of Essex, England, and LEONARD PHILIP WILSON, a subject of the King of Great Britain, residing at "Rosenmont," Holyhead Road, Coventry, in the county of Warwick, England, have invented 10 new and useful Improvements in the Manufacture and Production of Cellulose Compounds, of which the following is a specification.

In the manufacture of viscose, or solutions 15 of sodium cellulose xanthate, alkali cellulose is first made by steeping cellulose in a solution of caustic soda of about 1.2 specific gravity. The surplus soda solution is then removed and the mass of alkali cellulose is 20 disintegrated and, as a rule, packed in boxes, to mature or "mercerize." The period of maturing, or "mercerizing," and the temperature at which it takes place (generally between 15° and 25° centigrade) determine 25 the viscosity of the viscose and must be varied with the different qualities of cellulose used.

It has hitherto been supposed that the 30 changes which take place are due to a slow direct action of the alkali upon the cellulose, that air has a prejudicial effect upon the reaction, and that a low temperature is requisite for storage and for obtaining satisfactory results, and the methods hitherto adopted in manufacture have been based 35 upon these suppositions. See, for example, Margosches in "Die Viscose", Leipzig, 1906, pages 41 and 42.

Alkali-cellulose has been packed in tightly closed vessels, containing preferably not 40 more than 100 kilos., in order to prevent the entrance of air and any spontaneous heating due to the exothermic nature of the reaction. The maturing process has generally occupied several days.

45 It has now been found that oxidation is an action essential to the changes which take place during the process of maturing, and that while, for instance, the required effect is not produced if cellulose (for example 50 wood-pulp) be completely immersed in the caustic soda solution for several days (a period which would be sufficient if, after a short immersion, the alkali cellulose were

exposed to the action of air in a more, or less, combined space) on the other hand, 55 treatment with caustic soda solution for a comparatively short time, say for about from four, to five, hours, is sufficient to complete the desired action if oxygen, or other suitable oxidizing agent be supplied, and 60 this invention consists in supplying an oxidizing agent which may be effected in any suitable way; for example, we may use a soluble peroxid, such as sodium peroxid, or hydrogen peroxid, or a mixture of such 65 peroxids, or a hypochlorite, or a current of oxygen, or inert gas, or gases, mixed with oxygen, or air may be used.

The following are examples of how this invention, having for its basis the treatment of alkali-cellulose with oxygen, or other suitable oxidizing agent, may be performed, but it is not limited to these examples.

### Example 1.

2 kilos of sodium peroxid are dissolved in 200 kilos of 17½ per cent. solution of caustic soda and 5 kilos of wood-pulp, in sheet form, are immersed in the liquid at a temperature of about 18° centigrade, for from four, to 80 five, hours. The product is then removed and pressed until it weighs about 15 kilos., after which it may be ground and at once converted into xanthate by the action of carbon bisulfid. 85

### Example 2.

Alkali-cellulose, which has been prepared from wood-pulp, and milled, in the manner usually adopted in the manufacture of viscose, is placed in a vessel, which is rotated and, by means of a water-jacket, kept at a temperature of 40° centigrade. After a short time, when the contents have acquired the same, or about the same, temperature as 90 that of the vessel, a steady current of air is blown through the contents for four hours. Cold water is then run through the jacket to cool the contents, and, when they have been reduced to a temperature suitable for xanthation, carbon bisulfid may be added and the conversion into viscose completed. 95

As stated, we do not limit ourselves to the particular ways described in these examples, for effecting the oxidation of alkali cellulose 100 according to this invention as it may be 105

2  
effected in other ways. For example, we  
may blow oxygen, or air, or a mixture of  
oxygen with air, or with inert gas, or gases,  
through the solution in which the cellulose  
5 is immersed, or through the heated alkali-  
cellulose, or we may expose large surfaces of  
the alkali-cellulose freely to the atmosphere  
in a room heated above 30° centigrade, but  
we do not claim the limited exposure of  
10 alkali-cellulose to the action of atmospheric  
air at temperatures of 30° centigrade and  
under, such as occurs in the maturing of  
alkali-cellulose in the usual manner.

When using oxidizing agents other than  
15 those hereinbefore named regard must be  
had to the question of the possibility of sec-  
ondary changes, or the formation of sec-  
ondary products, which, by reason of their  
color, insolubility, tendency to promote fur-  
20 ther changes, or otherwise, might, for the  
purpose in view, be objectionable. For ex-  
ample, if a solution of potassium permanganate  
(which is a suitable oxidizing agent in  
certain cases) be used, the insoluble brown  
25 hydroxid of manganese is formed and there-  
fore potassium permanganate should not be  
used in cases where such hydroxid would  
be objectionable.

By means of this invention the time re-  
30 quired to mature alkali-cellulose can be  
greatly reduced, for example to a few hours,  
while the process is brought more under con-  
trol, and kinds of cellulose which were pre-  
viously considered as unsuitable can be suc-  
35 cessfully used.

Although we have described this inven-  
tion more particularly with reference to the  
manufacture of viscose solutions, it is not  
limited thereto but includes the oxidation of  
40 alkali-cellulose as hereinbefore explained  
whether in the manufacture of viscose, or  
not.

By varying the time, or the temperature,  
of treatment, or the quantity of oxidizing  
45 agent employed, products of different de-  
grees of oxidation, and viscose solutions of  
various degrees of viscosity, and other qual-  
ties, can be obtained. The invention is emi-  
nently useful in the manufacture of artificial  
50 silk, but it is to be understood that the prod-  
ucts can be used for any purpose for which  
they are applicable.

It is to be understood that in the present  
specification and claims the term "alkali-  
55 cellulose" is used in its technical sense and  
should not be confused with the well known  
"soda-pulp." The basis of the invention is  
the discovery that cellulose when chemically  
60 combined with caustic soda in the form of  
what is known technically as "alkali-cellu-

lose" is particularly sensitive to oxidation  
and that a useful product can be so obtained.  
A typical alkali-cellulose is prepared by  
steeping cellulose in a solution of 17.5 per  
cent. caustic soda and pressing to about 65  
three times its original weight; so that it  
contains about fifteen (15) per cent. caustic  
soda and twenty-eight (28) per cent. cellu-  
lose. It is decomposed by the action of wa-  
ter into caustic soda solution and cellulose. 70

If a weak solution of about five (5) per  
cent. caustic soda be used to soak the cellu-  
lose and it is well pressed to remove surplus  
moisture, the cellulose does not combine ap-  
preciably with the alkali and the product is 75  
found to contain only from 2 to 3 per cent.  
caustic soda.

Alkali-cellulose is quite distinct from  
"soda-pulp" which contains no alkali and  
which has had the soda washed out after 80  
being boiled in it. To such a product as  
"soda-pulp" the invention and the subjoined  
claims do not relate.

What we claim is:—

1. In the manufacture of cellulose com-  
pounds, subjecting alkali-cellulose to oxida-  
tion by positively supplying thereto an ox-  
idizing agent. 85
2. In the manufacture of cellulose com-  
pounds, subjecting alkali-cellulose to oxida-  
tion by positively supplying oxygen thereto. 90
3. In the manufacture of cellulose com-  
pounds, effecting the oxidation of alkali-  
cellulose by positively passing oxygen in ad-  
mixture with other gas in contact therewith. 95
4. In the manufacture of cellulose com-  
pounds, effecting the oxidation of alkali-  
cellulose by acting upon it with oxygen at a  
temperature above 30° C. 100
5. In the manufacture of cellulose com-  
pounds, effecting the oxidation of alkali-  
cellulose by acting upon it with oxygen in  
admixture with other gas at a temperature  
above 30° C. 105
6. In the manufacture of alkali-cellulose,  
treating wood-pulp with caustic soda solu-  
tion of sufficient strength to form alkali-  
cellulose and an oxidizing agent. 110
7. The manufacture of viscose which con-  
sists in treating alkali-cellulose with an ox-  
idizing agent and converting the product into  
cellulose xanthate.

In testimony whereof we have signed our  
names to this specification in the presence  
of two subscribing witnesses.

WALTER HAMIS GLOVER.  
LEONARD PHILIP WILSON.

Witnesses:

ERNEST HARKER,  
STELLA BENSON.